

## UNITED STATES PATENT OFFICE

IRVING F. LAUCKS AND GLENN DAVIDSON, OF SEATTLE, WASHINGTON, ASSIGNEES TO  
I. F. LAUCKS, INC., OF SEATTLE, WASHINGTON, A CORPORATION OF WASHINGTON  
CONSTRUCTION UNIT OF WOOD PLIES BOUND BY VEGETABLE-PROTEIN ADHESIVES

No Drawing. Original application filed October 29, 1928, Serial No. 671,381. Patent No. 1,689,732.  
Divided and this application filed November 2, 1927. Serial No. 230,686.

This invention relates to a new article of manufacture, and more particularly a veneer construction unit involving wood plies bound by a vegetable protein adhesive.

The art of making a water-proof glue from certain protein materials has been known for some time; thus casein and blood albumin are in common use. These last mentioned compounds, however, have a number of disadvantages from a practical standpoint. Casein is costly and lack of uniformity in the material as derived from various sources is a serious detriment; while blood albumin is not available except in certain situations. There is accordingly a great demand, particularly in the veneer industry where large quantities of glue are consumed, for a new glue that will be cheap and at the same time sufficiently water-proof.

By water-proof, in this connection, it is not meant that glues thus characterized will resist the action of water indefinitely, but it is meant that they are water-proof in the sense in which the term is used in the veneer industry, viz., that a panel can be soaked in cold water for from seventy-two to one hundred hours, or in boiling water for eight hours, without separation.

Vegetable compounds have not, so far as we are aware, been heretofore satisfactorily employed as a basis for water-proof glues of the type in question. It is true that some veneer makers, on account of the high price of casein, have come to use starch glues but these, at least as heretofore made, are not at all water-proof, and vegetable proteins have not heretofore been used at all, so far as we are aware.

We have now discovered, however, that by subjecting the same to proper treatment, such vegetable proteins or vegetable matter containing proteins, can be converted into a water-proof glue that will satisfy the rigid requirements of veneer or plywood making. The requisite raw material may be derived from a number of sources and the treatment of such material is relatively simple and inexpensive not requiring an elaborate hot-pressing plant so that as a result we are able to produce a satisfactory product at a much

lower cost than has heretofore been possible.

To the accomplishment of the foregoing and related ends, the invention, then, consists of the features of combination hereinafter fully described and particularly pointed out in the claims, it being understood that such constitute but several of the various ways in which the principle of the invention may be used.

We have found that soya bean flour constitutes an admirable raw material for our purpose. Such flour is preferably made by grinding soya bean cake so that 80 per cent will pass a 100 mesh screen and when treated with certain chemicals, or other substances, we make therefrom a very satisfactory glue that meets the requirements of the veneer trade fully and is in many respects better than the usual glues now on the market. Such bean cake, as analyzed by us, is found to contain on the average 45 per cent protein, 12 per cent water, 5 per cent cellulose or crude fiber, 7 per cent oil, 6 per cent ash, and 25 per cent carbohydrates.

We do not, however, wish to limit ourselves to soya bean flour or to vegetable protein derived from this source for we have made satisfactory glue by our improved process from a low grade wheat containing approximately 10 per cent protein, and there are many other vegetable materials containing protein in amounts intermediate between the percentages thus noted as found in such soya bean flour and wheat or even lower than the percentage in such wheat that may be utilized with satisfactory results; that is, soya bean flour gives the best results, but other sources of vegetable protein-containing material may be employed with proportionately advantageous results.

Where employing a leguminous or vegetable seed flour we have an advantage not only in the protein content but also any gummy or other constituents. Besides, expensive separations and purifications are then not necessary.

Soya bean flour made from soya bean cake from which the oil has been expressed, is preferably used in practice because it is cheaper and makes a better glue, but flour

made from whole soya beans, without expressing the contained oil, may also be used, although obviously this would not be economical in view of the value which attaches to such oil. As to the fineness of the flour, it is not necessary that the meal be ground as fine as indicated above, but fineness is desirable from a practical standpoint.

Preferably we react on our vegetable protein-containing material with both caustic soda and lime. As equivalents of such caustic soda, caustic potash and ammonia may be used, although more expensive. Other equivalents of caustic soda are salts of soda 15 (or potash) with weak acids, e. g. sodium phosphate, sodium borate and the like. Similarly in place of lime, magnesia, baryta and strontia may be used as equivalents.

In order to improve the working properties, e. g. the spreading and flow, of the glue produced as aforesaid as well as the water resisting properties, we have found it desirable to add other substances of which the following are examples:—

25 Carbon bisulfide, calcium polysulfide. Equivalents would be other sulfur compounds of like properties or constitution which bring about or impart water-resisting properties, these being more particularly sulphur-containing compounds which provide a sulphur derivative of carbonic acid.

Silicates, preferably sodium silicate.

We have also found that certain substances will act in the same way as the caustic soda 35 and also as thinners, e. g. sodium phosphate, sodium perborate and sodium sulphite. These salts are all related in that they are combinations of the strong base sodium with a weak acid and there are a number of other 40 salts that fall in the same category and which have a similar effect, so need not be listed in detail.

As examples we may cite the following typical formulæ:—

45 (1) Mix 30 parts soya bean flour with 120 parts water; add 13 parts of 18 per cent caustic soda solution and mix; 5 parts carbon bisulfide are then added and stirred well; to this 3 parts calcium hydrate are added and 50 stirred in; then 15 parts water glass (sodium silicate) are stirred in; finally, add 1 part copper sulfate to 5 parts of water and stir in. This makes the finished glue, which is then spread on panels, for example, put under pressure in convenient stacks or presses for several hours, whereupon the pressure 55 may be released.

(2) Mix 30 parts soya bean flour, 1 part alum, 70 parts water; add 13 parts 18 per cent caustic soda solution and 4 parts calcium hydrate in 20 parts water.

(3) Mix 30 parts low grade wheat flour, 10 parts Portland cement, 30 parts water, 30 parts 18 per cent caustic soda solution; warm 65 to 80 degrees cent.; add 15 parts water glass.

The particular order in which the several ingredients are mixed together in the formulæ just given may be varied, and it is not necessary that the manufacture of the adhesive be completed in a single continuous 70 operation, but as a matter of practice we have found it desirable in certain cases to mix only certain of the ingredients initially and then add the others just before the glue is required for use.

It will also be understood, of course, that the foregoing formulæ are typical and that many variations are actually made therein in the compounding of our improved glue.

This application is a division of our application, Serial No. 671,381, filed Oct. 29, 1923.

Other modes of applying the principle of our invention may be employed instead of the one explained, change being made as regards 85 the process herein disclosed or the materials employed in carrying out such process provided the stated ingredients and steps or the equivalent of such stated ingredients or steps be employed.

We therefore particularly point out and distinctly claim as our invention:—

1. In a laminated construction unit, wood in layer form bound resistively against water separation by a water-withstanding composition including the reaction products of leguminous seed flour, caustic soda and lime.

2. In a laminated construction unit, wood in layer form bound resistively against water separation by a water-withstanding composition including the reaction products of ground soya bean cake, caustic soda and lime.

3. In a laminated construction unit, wood in layer form bound resistively against water separation by a water-withstanding composition including the reaction products of leguminous seed flour, caustic soda and a copper compound.

4. In a laminated construction unit, wood in layer form bound resistively against water separation by a water-withstanding composition including ground soya bean cake, caustic soda and a copper compound.

5. In a laminated construction unit, wood in layer form bound resistively against water separation by a water-withstanding composition including the reaction products of leguminous seed flour, caustic soda, lime and copper sulphate.

6. In a laminated construction unit, wood in layer form bound resistively against water separation by a water-withstanding composition including ground soya bean cake, caustic soda, lime and copper sulphate.

7. In a laminated construction unit, wood in layer form bound resistively against water separation by a water-withstanding composition including the reaction products of leguminous seed flour, caustic soda, lime, copper sulphate and sodium silicate.

8. In a laminated construction unit, wood in layer form bound resistively against water separation by a water-withstanding composition including the reaction products of ground soya bean cake, caustic soda, lime, copper sulphate and sodium silicate.
9. As an article of manufacture, a veneer construction unit comprising a plurality of wood plies bound together by a waterproof adhesive including the reaction products of a vegetable protein, an alkaline medium, and a sulphur-containing agent.
10. As an article of manufacture, a veneer construction unit comprising a plurality of wood plies bound together by a waterproof adhesive including the reaction products of a vegetable protein, an alkaline medium, and carbon bisulphide.
11. In a laminated construction unit, a wooden ply bound by a waterproof adhesive including the reaction products of a leguminous seed flour and carbon bisulphide.
12. In a laminated construction unit, a wooden ply bound by a waterproof adhesive including the reaction products of soya bean flour and carbon bisulphide.
13. In a laminated construction unit, a wooden ply bound by a waterproof adhesive including the reaction products of soya bean protein with an alkali and a sulphur-containing compound.
14. As an article of manufacture, a veneer construction unit comprising a plurality of wood plies bound together by a waterproof adhesive including the reaction products of soya bean protein and a sulphur-containing agent.
15. As an article of manufacture, a veneer construction unit comprising a plurality of wood plies bound together by a waterproof adhesive including the reaction products of soya bean protein and carbon bisulphide.
16. As an article of manufacture, a veneer construction unit comprising a plurality of wood plies bound together by an interposed adhesive including the reaction products of a vegetable protein-containing flour, caustic soda, carbon bisulphide, calcium hydrate, sodium silicate, and copper sulphate.
17. As an article of manufacture, a veneer construction unit comprising a plurality of wood plies bound together by an interposed adhesive including the reaction products of soya bean flour, caustic soda, carbon bisulphide, calcium hydrate, sodium silicate, and copper sulphate.

Signed by me, this 21st day of October, 1927.

IRVING F. LAUCKS.

Signed by me, this 29th day of October, 1927.

GLENN DAVIDSON.